

July 3, 1951

C. W. MONTGOMERY ET AL

2,559,457

## HYDRODESULFURIZATION OF PETROLEUM HYDROCARBONS

Filed May 2, 1949



INVENTORS  
CHARLES W. MONTGOMERY  
WILLIAM J. GILBERT  
STANLEY M. HAZEN

BY F.M. Haughton  
~~their~~ ATTORNEY

## UNITED STATES PATENT OFFICE

2,559,457

HYDRODESULFURIZATION OF PETROLEUM  
HYDROCARBONS

Charles W. Montgomery and William I. Gilbert,  
Oakmont, and Stanley M. Hazen, Indiana  
Township, Allegheny County, Pa., assignors to  
Gulf Research & Development Company, Pitts-  
burgh, Pa., a corporation of Delaware

Application May 2, 1949, Serial No. 90,864

5 Claims. (Cl. 196—28)

1

This invention relates to the hydrodesulfurization of petroleum hydrocarbons and more particularly to a method of contacting sulfur-bearing petroleum hydrocarbons in the presence of hydrogen with a contact agent to remove the sulfur therefrom.

Among the most efficient methods of processing high sulfur petroleum hydrocarbons is the contact or absorption desulfurization process. This procedure is described in U. S. application Serial Nos. 699,671 and 699,672, filed September 27, 1946, by W. A. Horne and J. F. Junge, now respectively Patent Nos. 2,516,876 and 2,516,877 of August 1, 1950, and comprises contacting high sulfur content petroleum hydrocarbons with a contact comprising iron group metals and/or metal oxides on a carrier in the presence of hydrogen. This process has proved to be highly successful and is believed to be the most efficient type process for the removal of sulfur from high sulfur crude and gasolines. However, we have found that when the process is repeated and the contact regenerated for long periods, the contact tends to decrepitate. This problem assumes large proportions with the contact type hydrodesulfurization process in as much as it involves frequent regeneration of the contact due to the carbon lay down as a result of the action of the iron group metal or oxide. Due to this decrepitation the contact tends to lose its efficacy after repeated regeneration and use since the pulverization of the contact induces an excessive pressure drop across the contact bed. Ultimately this requires a shut-down of the process and consequent replacement of the catalyst bed with concomitant expense and loss of production time.

This invention has as an object the provision of a contact hydrodesulfurization process in which there is a marked decrease in the amount of contact pulverization.

A further object of the present invention is to provide a contact hydrodesulfurization process in which numerous regenerations may be carried out without replacing the contact bed.

Other objects will appear hereinafter.

These and other objects are achieved by the process of the present invention which comprises removing sulfur from petroleum hydrocarbons by contacting vapors of sulfur containing petroleum hydrocarbons and hydrogen-containing gas with a contact comprising a carrier on which has been deposited a mixture of nickel and/or nickel oxide and copper and/or copper oxide with the weight per cent of copper to nickel in the mixture being between 5 and 11 per cent, absorbing sulfur

2

from the vapors to form nickel and copper sulfide on the contact, and continuing said process until regeneration of the contact proves necessary, then regenerating said contact to substantially its original form and again contacting the vapors of the petroleum hydrocarbon and hydrogen containing gas with the regenerated contact.

As shown in the aforementioned Horne and Junge applications the hydrodesulfurization is accomplished at varying temperatures, pressures and space velocities with the optimum conditions depending on the type charge stock that is used. For example, with low boiling hydrocarbons such as those normally liquid petroleum fractions having an ASTM end point up to 600° F. such as straight run or cracked gasolines and naphtha, the temperature will usually lie between 600° and 800° F. At temperatures below 600° F., the desulfurization activity of the contact diminishes whereas with temperatures higher than 800° F. excessive cracking reactions result in decreased product recovery and rapid coke formation which deactivates the contact. We have further found that the optimum pressures lie between 100 and 500 p. s. i. g. At pressures below 100 p. s. i. g. the partial pressure of hydrogen is not sufficient to maintain desulfurization activity nor to suppress cracking reactions which result in coke formation. Increasing the pressure above 500 p. s. i. g. results in only a slight incremental gain in desulfurization, and a decrease in the bromine number of the end product gasoline and is thus not commercially desirable. The preferred space velocities lie between 0.2 and 6.0 liquid volumes of charge per hour per volume of contact agent. Space velocities below 0.2 result in excessive cracking and olefin saturation reactions caused by the long contact time whereas at space velocities above 6.0 the contact time is too short to provide sufficient desulfurization.

The foregoing conditions are applicable to the treatment of low boiling hydrocarbons. However this invention can be applied with exceptional success to high boiling petroleum hydrocarbon oil such as total crude as well as topped or reduced crude. These terms may be defined as follows: "total crude" is defined as naturally occurring petroleum oil which has not been processed in any manner but has been or preferably should be separated from water or sediment and desalinated. "Topped or reduced crude" is defined as the residual petroleum oil resulting from removal of all or some of the straight run fractions such as gas, gasoline, kerosene, naphtha, furnace oil, gas oil, etc. which are normally re-

moved from the above-defined total crude by the process of atmospheric and/or vacuum topping or distillation. Charge stocks such as total crude which has been diluted or admixed with lower boiling straight run or cracked petroleum fractions including gases are also included. Diluents of this kind may be required in processing low gravity crudes such as some of those from Mississippi as well as those from Kuwait. Diluents may also be necessary and preferred in desulfurizing topped or reduced crudes. The purpose of this diluent is to assist vaporization of the heavier constituents of the charge stock. In some cases it may be desirable to admix steam with the charge stock to assist vaporization. Preferred operating conditions for the aforementioned high boiling petroleum hydrocarbons may vary within certain ranges depending upon the charge stock.

We have found the optimum temperature range to be from 750° to 950° F. for high boiling petroleum hydrocarbons. At temperatures below 750° F. the desulfurizing activity of the contact diminishes whereas at temperatures greater than 950° F. excessive cracking actions result in decreased product recovery and rapid coke formation which deactivates the contact. We have further ascertained the preferred pressure range to be between 100 and 1000 p. s. i. g. With pressures below 100 p. s. i. g. it appears that the partial pressure of hydrogen is not sufficient to maintain desulfurizing activity nor to suppress cracking reactions which result in coke formation. Increasing the pressure above 1000 p. s. i. g. results in only a slight incremental gain in desulfurization and is thus not commercially desirable. The space velocity range which we prefer to employ is 0.2 to 6.0 volumes of charge per hour per volume of contact agent. A space velocity below the former causes excessive cracking reactions due to the long contact time, while space velocities above 6.0 are too short to allow sufficient desulfurization. As shown in these aforementioned Horne and Junge applications the hydrogen to oil ratio should be above 300 SCF/bbl.

The copper-nickel-carrier contacts of this invention may comprise copper and nickel in their metallic state, or in the state of their oxides, or as a mixture of the metallic and oxide states. A suitable method for preparing the metallic type contact is to impregnate a carrier such as alumina, kieselguhr, silica gel, aluminum silicates, silica-aluminas, Alfrax, Magnesol, Porocel, bauxite, diatomaceous earth, etc., with a combination solution or solutions of soluble salts of nickel and copper. Suitable soluble salts of nickel include the acetates, nitrates and nitrites. Suitable copper salts include the acetates, nitrates and nitrites. The concentration of these salts is adjusted so that the requisite amount of nickel and copper is deposited upon the carrier. The carrier is then dried, calcined and reduced by a suitable reducing gas such as a hydrogen-containing gas so that the nickel and copper are present on the carrier in their metallic states. If the oxide-type contact is desired, the above-mentioned impregnation technique may be utilized except that the reducing step is omitted.

The mixture of metallic and metal-oxide type contact is prepared by the identical treatment given for the preparation of the metallic type contact, except that the reduction is controlled so that but a portion of the nickel and copper is reduced to the metallic state.

It is to be understood that the above mentioned

methods of preparing the contact are not to be considered as all-inclusive and that other methods such as repeated coimpregnation or coprecipitation, readily apparent to one skilled in the art may be employed.

The following examples illustrate a method of preparing a conventional contact, and also for preparing a contact useful in applicants' invention. Example I indicates a method of preparing a contact in which nickel alone is present while Example II illustrates a method of preparing a contact of the type utilized in the present invention containing both nickel and copper.

*Example I.*—Contact A was prepared using 4 to 10 mesh Alorco granular "F-10" alumina which has a surface area of about 119 square meters per gm. The alumina base was placed in an evacuated chamber and a solution of nickel nitrate containing 20 per cent nickel oxide as nitrate was introduced so as to completely cover the alumina. After 5 minutes of impregnation under vacuum, the vacuum was broken and the alumina was allowed to stand for 10 more minutes in the nickel nitrate solution. At the end of this time, the nickel nitrate solution was drained from the contact. The contact was placed in an oven and dried in a stream of air at 248° F. for 46 hours. The temperature of the dried contact was then raised to 1000° F. over a period of about 6 hours and held at this temperature for an additional 10 hour period while a stream of air was passed over the contact. At this point the contact contained 13.3 per cent nickel oxide (or 10.8 per cent nickel on reduced basis). After cooling to room temperature, the above procedure was repeated, and, after calcining and cooling, the nickel oxide content was 22.1 per cent (or 18.25 per cent nickel on reduced basis). A third impregnation was carried out as above except that the nickel nitrate solution used for this impregnation contained 10 per cent nickel oxide as nitrate. After calcining and cooling, the contact was found to contain 25.1 per cent nickel oxide (or 20.8 per cent nickel on reduced basis). This is equivalent to 19.7 weight per cent nickel in the oxide form of the contact.

*Example II.*—Contact B was prepared from Alorco granular alumina "F-10" having a surface area of about 119 square meters per gm. and was 8 to 14 mesh in size. 350 cc. of the alumina base was calcined in a stream of nitrogen at 1000° F. for 2 hours. An aqueous solution of nickel nitrate containing 20 per cent nickel oxide was mixed with an aqueous solution of copper nitrate containing 20 per cent copper oxide so that the mole ratio of nickel oxide to copper oxide was 4 to 1. The calcined alumina base, after cooling to room temperature, was immersed for 15 minutes in the above nickel nitrate-copper nitrate solution. The solution was then removed from the contact and the contact was allowed to drain for 3 minutes. Vacuum was then applied for 5 minutes to further reduce the water content of the contact. The impregnated contact was placed in a furnace at 230° F. for 8 hours in a slow stream of nitrogen. After this drying period, the temperature of the contact in the furnace was brought to 1000° F. in 2 hours, while a slow stream of air was passed through the furnace. The contact was held at 1000° F. for 2 additional hours. After cooling to room temperature, the impregnated alumina was again immersed, drained, dried, and calcined as above. This procedure was carried out a third time, and after calcining, the nickel content of the con-

tact was 17.6 per cent and the copper content was 1.4 per cent, both metals being present in the form of the oxide.

In most cases the on-stream cycle should be terminated when hydrogen sulfide appears in substantial amounts in the effluent. This has been found to occur when about 30 to 60 per cent of the metallic content of the contact has been converted into sulfide. At this point the contact should be regenerated. In situations in which the commercial economics of the process permit the removal of relatively small amounts of hydrogen sulfide from the product the reaction may be continued until the metallic content of the contact has been completely converted into metallic sulfide before commencing regeneration.

The contacts of this invention may be regenerated by any of the well known prior art methods. However, this regeneration may best be accomplished by first purging the contact with an inert gas or steam in order to recover valuable hydrocarbons remaining in the contact bed. Following this purge the contact is regenerated through the use of an oxygen-containing gas such as air or oxygen. This forms sulfur dioxide gas which may be recovered by use of conventional methods, such as by solvent absorption and stripping. The further treatment of the contact will be dependent upon the type of contact. With oxide type contacts no further treatment beyond the aforementioned oxidation step need be employed. However, when the contacts comprise copper and nickel in the metallic state or as a mixture of metallic and oxide states, a reducing treatment to restore the contact to its original form is necessary.

The contacts of this invention may be used in numerous methods. Multiple or single fixed-bed systems may be utilized as well as an arrangement in which the contact is continuously charged and removed from the reaction zone and followed by external regeneration. Furthermore, the contact may be fragmentized into fine particles and utilized in a fluidized state.

Hydrodesulfurization runs were made to determine the relative hydrodesulfurizing activity of the contact containing nickel (contact A) as compared to the contact of the present invention containing both nickel and copper (contact B).

**Example III.**—West Texas crude was passed over contact A (prepared in Example I) having 19.7 per cent nickel, as nickel oxide, on alumina at a space velocity of 1.0 volume of charge per hour per volume of contact, and a temperature of 850° F., a pressure of 500 pounds per square inch, a hydrogen to oil ratio of 2000 SCF/bbl. for a throughput of 4.0. The sulfur content of the treated crude was 80 per cent less than that of the original crude.

A similar run was made under the identical conditions described above utilizing contact B (prepared in Example II) having a content of 17.6 per cent nickel, as nickel oxide, and 1.4 per cent copper, as copper oxide on an alumina support. There was a desulfurization of about 70 per cent, as compared with the 80 per cent desulfurization obtained with contact A having no copper.

It can be seen that the presence of copper decreases the hydrodesulfurization activity to a certain extent but for practical purposes, the falling-off of hydrodesulfurization activity does not become a serious problem as long as the hydrodesulfurization rate is above about 50 per cent.

cent, and hence the contacts of this invention serve as excellent hydrodesulfurization contacts.

In order to compare the powdering rate of the contacts of this invention which contain both copper and nickel with contacts in which the copper is omitted, and in order to show the critical nature of varying the weight per cent of copper based on the nickel content, the following experimental runs were made.

**Example IV.**—Applicants have found that the following test is an accurate method of determining the powdering rate of hydrodesulfurization contacts.

Normal heptane was passed with equimolar proportions of hydrogen over a bed of contact pellets. The apparatus that was utilized consisted of a 1 1/4" OD Pyrex tube surrounded by an electrically heated furnace. In the bottom of the tube was placed a plug of glass wool and on top of the glass wool 50 cc. of contact pellets of about 1/8" diameter. Above the pellets was placed an approximately equal volume of Pyrex chips. When the Pyrex chips and contact pellets had reached the desired temperature, metered hydrogen and normal heptane were introduced at the top of the Pyrex tube and allowed to flow downward over the Pyrex chips and then over the contact pellets. The effluent from the bottom of the Pyrex tube passed through a condenser and then into a carbon dioxide-acetone-cooled trap where the liquid products were accumulated. The gases passed out of the trap through a wet test meter. At the end of each run the Pyrex chips were removed from the tube and the total weight and volume of the contact were determined. The contact material was then screened to separate the fines from the pellets, and the weight and volume per cent fines were determined.

The temperature was 850° F., the gaseous space velocity being 590 cc./hr./cc. catalyst at standard temperature and pressure, with the actual flow rate of hydrogen being  $9.9 \times 10^{-3}$  ft.<sup>3</sup> per min. and that of the heptane being 1.7 cc./min. (liq.), or a value of 0.011 mol/min. for both the hydrogen and the heptane. The amount of catalyst charge in each run was 50 cc.

The following table discloses the powdering rates for each contact, e. g. powdering rates

| Run | Type                                   | wt. of fines in gms. $\times 100$         |         | Percent Cu based on Ni | Powdering Rate W |
|-----|----------------------------------------|-------------------------------------------|---------|------------------------|------------------|
|     |                                        | wt. of catalyst charge + deposited carbon | minutes |                        |                  |
| 55  |                                        | Percent metal reduced bases               |         |                        |                  |
|     |                                        | Ni                                        | Cu      |                        |                  |
| 1   | NiO-Al <sub>2</sub> O <sub>3</sub>     | 22.01                                     | 0       | 0                      | 3.37             |
| 2   | NiO-CuO-Al <sub>2</sub> O <sub>3</sub> | 21.62                                     | 1.39    | 6.44                   | 2.25             |
| 3   | NiO-Al <sub>2</sub> O <sub>3</sub>     | 10.5                                      | 0       | 0                      | 2.076            |
| 4   | NiO-CuO-Al <sub>2</sub> O <sub>3</sub> | 8.41                                      | 2.32    | 27.6                   | 0                |
| 5   | do                                     | 9.13                                      | 1.10    | 12.2                   | 0                |
| 6   | do                                     | 9.58                                      | 0.55    | 5.75                   | 0.143            |
| 7   | do                                     | 9.84                                      | 0.22    | 2.24                   | 1.004            |

Figure 1 was prepared from data similar to runs 4, 5, 6, and 7 in order to reveal the variation of the powdering rate "W" with the change in weight per cent of copper based on the weight of nickel.

It should be noted that the absolute powdering rate will be a function of the total amount of metal present in the contact (as shown by a comparison of runs 1 and 2 with runs 3 to 7), as well as the weight per cent of copper based on nickel. However, for a given total metal content

the relative powdering rate will vary with the weight per cent of copper. This is readily apparent from a comparison of run 1 with run 2, and runs 3 to 7 with each other.

Figure 1 was prepared from data similar to the foregoing and illustrates the decrease in powdering rate concomitant with an increase in the per cent of copper up to the value of about 11 or 12 weight per cent based on nickel. Furthermore, from a consideration of the data presented in Example IV, runs 3, 6 and 7, and especially from accompanying Figure 1, it can clearly be seen that the powdering rate of contacts in which the copper is omitted is vastly greater than those in which it is present. In addition, it is apparent that the maximum change of slope of the powdering rate curve occurs at the value of about 5 weight per cent copper, and that the powdering rate increases rapidly when the percentage copper is reduced below this value. Thus, this value is to be regarded as the critical minimum value, that is the lowest value at which the addition of copper to the contact has a substantial effect on powdering rate. Also it is readily evident from Figure 1 that increasing the percentage of copper beyond 11 per cent has no effect on the powdering rate, since the powdering rate at the value of 11 weight per cent copper is nil.

Further hydrodesulfurization runs were conducted in order to determine the effect of adding additional copper to the contact beyond that required to reduce the powdering rate.

*Example V.*—Utilizing conditions similar to those given in Example III, hydrodesulfurization runs were conducted with contacts having varying weight per cent copper values based on nickel. The through-put at which hydrogen sulfide appeared, i. e. the volume of charge stock/volume of contact/cycle, and in which the cycle is defined as the duration of time from the point when the reaction was commenced till the time at which hydrogen sulfide appeared, was determined for each contact as follows:

| Weight percent Copper Based on Nickel | Through-put at which Hydrogen Sulfide Appears |
|---------------------------------------|-----------------------------------------------|
| 0                                     | 4                                             |
| 8.16                                  | 3                                             |
| 16.7                                  | 2                                             |
| 33.6                                  | 1.5                                           |

It will be seen that there is a decrease in the through-put on increasing the amount of copper. For this reason it is undesirable to use any more copper than is necessary to suppress powdering of the contact. Data similar to the foregoing were plotted and appear in accompanying Figure 2 wherein it is seen that with increasing amounts of copper the through-put decreases in a more or less incremental manner.

As a practical matter it is not desirable to decrease the through-put, but the desirability of decreasing the powdering rate greatly outweighs the loss of through-put. Hence, it may readily be observed from a consideration of Examples IV and V that increasing the weight per cent of copper beyond about 11 or 12 per cent based on nickel will not result in any greater beneficial decrease in the powdering rate, but will adversely affect the through-put values.

The aforementioned results illustrate the antagonistic relationship obtained on adding copper to nickel to form a hydrodesulfurization

contact agent. Thus, below the value of about 5 weight per cent copper based on nickel, the powdering rate of the contact is excessive, whereas above about the 11 per cent value it is nil; and furthermore increasing the copper content above about 11 per cent causes the through-put to adversely decrease. It can therefore be seen that the range 5 to 11 weight per cent of copper based on nickel is a critical one comprising that at which the powdering rate is decreased to a point where it does not impair the efficiency of the process, and at which the decrease of the through-put is not sufficiently marked to hamper the on-stream cycle.

In addition to the foregoing, it was also observed that on increasing the weight per cent of copper based on nickel the per cent hydrodesulfurization decreased.

*Example VI.*—Utilizing conditions similar to those given in Example III hydrodesulfurization runs were conducted with the following contacts. In the following table the per cent hydrodesulfurization that was obtained with each contact is indicated.

| Percent Ni Based on Contact | Percent Cu Based on Contact | Percent Cu Based on Ni | Percent Hydrodesulfurization |
|-----------------------------|-----------------------------|------------------------|------------------------------|
| 16.98                       | 0                           | 0                      | 76.5                         |
| 17.50                       | 1.43                        | 8.16                   | 58.8                         |
| 15.10                       | 2.52                        | 16.7                   | 55.1                         |

From the foregoing it is evident that the falling off of hydrodesulfurization concomitant with the increase in copper content does not result in a reduction to a value that would impede the commercial practicability of the process, because as heretofore stated contacts having above about 50 per cent hydrodesulfurization values are industrially serviceable. However, it can be seen that increasing the weight per cent of copper based on nickel causes the hydrodesulfurization activity of the contact to decrease and hence is undesirable.

Thus, it is to be emphasized that while increasing the weight per cent of copper based on nickel beyond the 11 per cent value fails to produce a further beneficial decrease in the powdering rate, adverse effects upon the through-put and the hydrodesulfurization activity of the contact will be obtained. Accordingly, it is essential for the purposes of the present invention to limit the weight per cent copper based on nickel to a value of between about 5 and 11 per cent.

The results achieved by the present invention are a function of the ratio of the weight per cent of copper to nickel and will be more or less independent of the total amount of metal which may be present. However, we have found that for the present process to be commercially applicable the total weight of metal in the contact should be from between about 5 to about 25 per cent. In addition to the copper and nickel, minor amounts of other metals may be present, such as iron, cobalt, calcium, and magnesium.

We do not wish to be bound by any theory for the present invention, however, we believe that the powdering is caused by the deposition of carbon from the hydrocarbon compounds which are being treated. The copper evidently prevents the carbon from entering the metal crystal lattice of the contact and thereby prevents the powdering and decrepitation heretofore encountered with these contacts.

The present process permits an increase in the production time for which a given catalyst bed may be utilized, and furthermore will permit a given hydrodesulfurization contact to be regenerated more frequently than has heretofore been possible. This means a marked saving in both time and money when our contact hydrodesulfurization process is utilized, as well as ease of operation.

We claim:

1. In the process for desulfurizing a petroleum hydrocarbon by contacting vapors thereof and hydrogen-containing gas with a contact comprising a member of the group consisting of nickel and nickel oxide on a carrier, absorbing sulfur from the vapors to form nickel sulfide, regenerating the contact to substantially its original form and again contacting the petroleum hydrocarbon vapors and hydrogen with the regenerated contact, the improvement for reducing powdering of said contact as a result of repeated regeneration which comprises incorporating copper in said contact in an amount of between 5 and 11 per cent by weight of the nickel whereby powdering is effectively reduced.

2. In the process for desulfurizing a high boiling petroleum hydrocarbon by contacting vapors thereof and hydrogen-containing gas with a contact comprising a member of the group consisting of nickel and nickel oxide on a carrier, at a temperature between 750° and 950° F., absorbing sulfur from the vapors to form nickel sulfide, regenerating the contact to substantially its original form and again contacting the petroleum hydrocarbon vapors and hydrogen with the regenerated contact, the improvement for reducing powdering of said contact as a result of repeated regeneration which comprises incorporating copper in said contact in an amount of between 5 and 11 per cent by weight of the nickel whereby powdering is effectively reduced.

3. In the process for desulfurizing a petroleum hydrocarbon by contacting vapors thereof and hydrogen-containing gas with a contact comprising a member of the group consisting of nickel and nickel oxide on a carrier the per cent nickel in the entire contact being between 5 and 25 per cent, absorbing sulfur from the vapors to form nickel sulfide, regenerating the contact to substantially its original form and again contacting the petroleum hydrocarbon vapors and hydrogen with the regenerated contact, the improvement for reducing powdering of said contact to

tact as a result of repeated regeneration which comprises incorporating copper in said contact in an amount of between 5 and 11 per cent by weight of the nickel whereby powdering is effectively reduced.

5 4. In the process for desulfurizing a high boiling petroleum hydrocarbon by contacting said hydrocarbon and hydrogen-containing gas with a contact comprising a member of the group consisting of nickel and nickel oxide on a carrier the per cent nickel in the entire contact being between 5 and 25 per cent, absorbing sulfur from the high boiling hydrocarbon to form nickel sulfide, regenerating the contact to substantially its original form and again contacting the high boiling petroleum hydrocarbon and hydrogen with the regenerated contact, the improvement for reducing powdering of said contact as a result of repeated regeneration which comprises incorporating copper in said contact in an amount of between 5 and 11 per cent by weight of the nickel whereby powdering is effectively reduced.

10 5. In the process for desulfurizing a high boiling petroleum hydrocarbon by contacting vapors thereof and hydrogen-containing gas with a contact comprising a member of the group consisting of nickel and nickel oxide on a carrier the per cent nickel in the entire contact being between 5 and 25 per cent, absorbing sulfur from the vapors to form nickel sulfide, regenerating the contact to substantially its original form and again contacting the petroleum hydrocarbon vapors and hydrogen with the regenerated contact, the improvement for reducing powdering of said contact as a result of repeated regeneration which comprises incorporating copper in said contact in an amount of about 11 per cent by weight of the nickel whereby powdering is effectively reduced.

20 40 CHARLES W. MONTGOMERY.  
WILLIAM I. GILBERT.  
STANLEY M. HAZEN.

#### REFERENCES CITED

45 The following references are of record in the file of this patent:

#### UNITED STATES PATENTS

| Number       | Name   | Date          |
|--------------|--------|---------------|
| 50 1,257,829 | Evans  | Feb. 26, 1918 |
| 2,073,578    | Gwynn  | Mar. 9, 1937  |
| 2,273,298    | Szayna | Feb. 17, 1942 |
| 2,337,358    | Szayna | Dec. 21, 1943 |